

Jan. 12, 1932.

J. E. PERRY ET AL

1,841,297

## APPARATUS AND METHOD OF CONTINUOUS CASTING OF STEEL

Filed April 26, 1928

6 Sheets-Sheet 1



INVENTORS  
*John E. Perry and*  
*George Ramsey*  
BY  
*George Ramsey*  
their ATTORNEY

Jan. 12, 1932.

J. E. PERRY ET AL

1,841,297

APPARATUS AND METHOD OF CONTINUOUS CASTING OF STEEL

Filed April 26, 1928

6 Sheets-Sheet 2



INVENTORS  
John E. Perry and  
George Ramsey  
BY  
George Ramsey  
ATTORNEY

Jan. 12, 1932.

J. E. PERRY ET AL.

1,841,297

# APPARATUS AND METHOD OF CONTINUOUS CASTING OF STEEL

Filed April 26, 1928

6 Sheets-Sheet 3

Fig. 3.



Fig. 4.



Fig. 5.



Fig. 6.

INVENTORS  
John E. Perry and  
George Ramsey  
BY  
George Ramsey  
the ATTORNEY

Fig. 7.

Jan. 12, 1932.

J. E. PERRY ET AL

1,841,297

APPARATUS AND METHOD OF CONTINUOUS CASTING OF STEEL

Filed April 26, 1928

6 Sheets-Sheet 4



INVENTORS  
John E. Perry and  
George Ramsey  
BY  
George Ramsey  
their ATTORNEY

Jan. 12, 1932.

J. E. PERRY ET AL

1,841,297

# APPARATUS AND METHOD OF CONTINUOUS CASTING OF STEEL

Filed April 26, 1928

6 Sheets-Sheet 5



INVENTORS  
*John E. Perry and*  
*George Ramsey*  
BY  
*George Ramsey*  
THE ATTORNEY

Jan. 12, 1932.

J. E. PERRY ET AL.

1,841,297

## APPARATUS AND METHOD OF CONTINUOUS CASTING OF STEEL

Filed April 26, 1928 6 Sheets-Sheet 6



INVENTORS  
*John E. Perry and  
George Ramsey*  
BY  
*George Ramsey*  
their ATTORNEY

## UNITED STATES PATENT OFFICE

JOHN E. PERRY, OF YOUNGSTOWN, OHIO, AND GEORGE RAMSEY, OF BROOKLYN,  
NEW YORK

## APPARATUS AND METHOD OF CONTINUOUS CASTING OF STEEL

Application filed April 26, 1928. Serial No. 272,925.

The present invention relates broadly to metallurgy and more especially to the metallurgy pertaining to steel.

Heretofore in the art of molten steel, in the primary step for fabrication, has been solidified by casting in ingot molds. In this practice individual quantities of molten steel are separated and permitted to cool and solidify into steel ingots. After the solidification of the ingot is complete, the ingot molds are stripped from the ingots and the ingots are placed in a soaking pit, where a reheating takes place. The ingots are then placed on a blooming mill table and run through the blooming mill, which forms the ingot into billets, blooms, slabs, or other intermediate shapes desirable for subsequent treatment. From the blooming mill the steel in its intermediate shape goes to the final fabricating mill, where the steel is rolled into sheets, bars, plates, rails, or such other form as the steel manufacturer is producing. Intermediate the several foregoing steps various shearing and reheating operations occur; for example, it is customary in the art to cut off or crop parts of the steel after it has passed the blooming mill, then this cropped material goes back as scrap, thereby adding to the expense of producing the final shapes.

The present invention comprises a method and apparatus which obviates all of the steps above enumerated between the ladle and the rolling mill. According to the present invention, the steel direct from the ladle is subjected to continuous treatment which results in a continuous longitudinal mass of solid steel of predetermined thickness, width and cross section, ready to immediately go into the rolling mill, whereby the treatment of the steel from the ladle to the finished product comprises a series of continuous operations without intermediate distinct separate steps.

In the preferred form of the invention the steel is formed into a pool which is continuously replenished from a ladle or ladles and the outlet of the pool is in one direction only, whereby the molten metal is carried along on chill members which in the initial stage chill the bottom and sides of the pool and in a

later stage chill the entire surface of the pool. At this moment the steel is in the condition of a wedge shaped molten core surrounded by solidified steel and with the base of the molten wedge being the open pool of molten steel. As the travel of the steel progresses the chilling and solidification continues inwardly and pressure on the steel is gradually increased so that the molten core gradually freezes solid and when the steel leaves this stage in the process it is completely solidified and comprises a continuously travelling mass of steel of a predetermined cross section. In the preferred form the cross section comprises a relatively flat continuous slab. This slab however has a shaped cross section to best suit the final shape to be rolled. This slab leaves the solidifying apparatus with sufficient initial heat to permit immediate rolling operations, thereby eliminating the soaking pit and the blooming mill for the reason that the shape given to the steel as it leaves the solidifying apparatus is such shape as the steel would have when it leaves the blooming mill. Where continuous operations are being performed this continuous slab immediately goes into the rolling mill. Where desired, shears may be interposed between the solidifying apparatus and the mill so that slabs of predetermined lengths may be cut from the solidified steel and the individual slabs may be treated, in rolling or forging, as individual units.

Where it is not necessary or desirable to shape the top of the slab, the method may be carried out by chilling from the bottom and sides only whereby the continuous stream of steel freezes from the bottom upward.

From the foregoing it will be observed that the present invention completely eliminates the ingot molds and all apparatus and manipulations necessary to casting in the ingot molds; the stripping apparatus, and all manipulations necessary for operating the stripping apparatus; the trackage, locomotive, buggies, and other conveying mechanism used for conveying the ingot mold and the ingot to and from the casting platform to the stripping mechanism and from the stripping mechanism to the soaking pit. It also

eliminates the soaking pit, the expense of fuel for reheating, the labor necessary to reheating, the mechanism, cranes, etc. for taking the ingots from the soaking pits to the blooming mill; the labor of handling the ingots in the blooming mill, the trouble, labor, expense and waste of cropping the ingots after passing the blooming mill, and other incidental mechanisms and apparatus necessary to carry out all of the foregoing intermediate steps between the ladle and the rolling mill as heretofore practiced in the art.

As heretofore practiced in the art, the large masses of steel which are cast in manufacturing large ingots for large shapes require several hours to crystallize, an average time being about eight hours from the time the ingot is poured until the time the ingot has passed through the blooming mill and is ready for rolling. In the present invention practically all of that time is saved and in a few minutes the molten steel from the ladle is solidified and ready for immediate rolling.

Other and further objects of the present invention will in part be obvious and will in part be pointed out hereinafter in the specification following.

It is realized that the invention may be embodied in and the methods may be practiced by apparatus other than that herein disclosed, and therefore the disclosure is to be understood as illustrative and not in the limiting sense.

Fig. 1 is a diagrammatic view illustrating an elevation of the preferred form of a solidifying and continuous slab casting mechanism.

Fig. 2 is a diagrammatic view illustrating a cross section taken on line 2-2 of Fig. 1.

Fig. 3 is a detail view illustrating a portion of the continuous mold members.

Fig. 4 is a perspective view of one of the mold members.

Fig. 5 is a diagrammatic view illustrating a portion of the mold top members.

Fig. 6 is a perspective view of one of the individual mold top members.

Fig. 7 is an end view of the mold top member illustrated in Fig. 6.

Fig. 8 and 9 illustrate cross sections of caps and molds to produce special shaped continuous slabs.

Fig. 10 and 11 illustrate cross sections of caps and molds to produce other special shapes, and wherein the thickness of the metal in caps and in the molds is arranged to produce predetermined chilling effects on the specially shaped continuous slabs.

Fig. 12 illustrates a mold and cap producing a continuous square billett.

Fig. 13 is a diagrammatic view of an apparatus in which the permanent dam at the front of the machine is replaced by inclining the bottom of the mold trough.

Fig. 14 is a diagrammatic plan view of the apparatus shown in Fig. 13.

Fig. 15 is a detail view of the pressure rail and roller for pressing the side members against the bottom of the mold trough illustrated in Figs. 13 and 14.

While the above method and apparatus and the invention disclosed herein are disclosed more particularly with reference to the steel art, it is to be understood that the invention is equally applicable to non-ferrous metals, which heretofore have customarily been cast in ingots or billets before being worked in final forms.

The apparatus disclosed herein diagrammatically comprises a steel solidifying device to which molten steel is supplied at one end and a solidified continuous steel slab is produced at the other end.

Referring now more especially to the drawings which diagrammatically illustrate in Figs. 1 to 7 a preferred form of the apparatus, a main drive shaft 1 carries a driving and supporting wheel 2 upon which is mounted a continuous mold trough 3 formed of individual mold members 4 which are suitably linked to each other so that when the mold members 4 are pushed through the machine the ends of these molds are tightly pressed together. This continuous mold trough 3 is supported at its upper run by driven rollers 5.

These driven rollers are preferably driven from the main drive shaft 1 by means of a large worm gear 6 which meshes with a driven worm gear 7 that turns a shaft 8 running the entire length of the machine. This shaft 8 carries bevelled gears 9 which mesh with roller bevelled gears 10 (two of these companion gears being shown in Fig. 1), whereby the continuous row of driven rollers 5 are all driven at the same rate. This series of driven rollers 5 forms a rolling bed on which the continuous mold trough 3 travels.

The continuous mold trough 3 after leaving the bed of driven rollers 5 passes over a supporting wheel 11 which is located near the output end of the machine. The lower run of the continuous mold trough 3 is supported upon a second set of driven rollers 12, which form a continuous under roller bed to support the molds on their return movement. These driven rollers 12 are likewise driven by a shaft 14 extending the full length of the under roller bed. This shaft 14 carries shaft 15 bevelled gears 16 which mesh with roller bevelled gears 17. The shaft 14 may be driven by a stub shaft 18 which carries on one end a worm gear 19 and on the other end a bevelled gear 20 that meshes with a bevelled gear 21 on the end of the shaft 14.

Near the front end of the machine is provided a dam member 22, which may comprise a relatively large block of iron or other suitable device. This dam 22 is intended to act as a chill member and if desired may be water cooled. The

Fig. 14 is a diagrammatic plan view of the apparatus shown in Fig. 13.

Fig. 15 is a detail view of the pressure rail and roller for pressing the side members against the bottom of the mold trough illustrated in Figs. 13 and 14.

While the above method and apparatus and the invention disclosed herein are disclosed more particularly with reference to the steel art, it is to be understood that the invention is equally applicable to non-ferrous metals, which heretofore have customarily been cast in ingots or billets before being worked in final forms.

The apparatus disclosed herein diagrammatically comprises a steel solidifying device to which molten steel is supplied at one end and a solidified continuous steel slab is produced at the other end.

Referring now more especially to the drawings which diagrammatically illustrate in Figs. 1 to 7 a preferred form of the apparatus, a main drive shaft 1 carries a driving and supporting wheel 2 upon which is mounted a continuous mold trough 3 formed of individual mold members 4 which are suitably linked to each other so that when the mold members 4 are pushed through the machine the ends of these molds are tightly pressed together. This continuous mold trough 3 is supported at its upper run by driven rollers 5.

dam 21 is located adjacent the initial straight part of the mold trough and substantially fits the inside of the mold trough by forming a relatively close contact with the sides and bottoms of the molds.

5 A pressure member comprising a continuous series of caps for the molds is arranged above the upper run of the continuous mold troughs in such manner as to allow a substantially open trough portion before the steel comes in contact with the capping members. The capping arrangement preferably comprises a continuous series 22 of individual caps 24 which are linked together to form a continuous chain. This continuous series of cap members is supported by a drive wheel 25 at one end of the continuous capping chain and a supporting wheel 26 at the other end thereof. The drive wheel 25 is also driven from the main drive shaft 1 by means of a worm gear 27 carried by shaft 28, and which worm gear 27 meshes with the main drive worm wheel 6. This shaft 28 at its opposite end carries a driving worm gear 29 that meshes with the worm gear 30 on the shaft of the drive wheel 25. This continuous series of caps is carefully timed to have a linear movement exactly according to the linear travel of the continuous mold trough 3 so that the caps for the molds move with the trough molds. The molds at this point comprise substantially a closed travelling tube in which the stream of molten steel is frozen into a continuously moving slab. Preferably the abutting ends of these 35 caps 24 are bevelled at 23 in order to maintain a tight joint between the caps as they come down on the molten steel when the caps are passing down around and off the periphery of the driving wheel 25. The lower run of the continuous series of caps is forced downwardly by means of a series of pressure rollers 31 which are so spaced that at all times two rollers are in contact with each cap, whereby the spaces between caps caused 40 by the bevelled ends do not cause an irregular pressure. Preferably, the axes of these pressure rollers are arranged in plane which gradually approaches the bottom of the continuous mold trough so that the pressure 45 rollers toward the forward end of the machine push the caps partly down against the molten steel in the traveling molds and by the time that the caps are at the rear end of the lower run of the continuous cap chain, the final pressure rollers 31 have firmly seated the caps upon the molds. These pressure rollers 31 may act as idler rolls except in very heavy duty machines where preferably they will be driven similarly to the mold supporting rollers 5, as heretofore described. The upper run of the continuous series of caps is also supported on supporting driving rollers 32 which assist the drive 55 wheel 25 in driving the cap chain. These

rollers 32 preferably are driven by means of a shaft 34 which carries a worm wheel 35 in contact with the worm gear 30 on the drive wheel shaft 25. The shaft 34 carries bevelled gears 36 (which are shown in Fig. 1) which mesh with bevelled gears 37 on the supporting driving rollers 32. An auxiliary set of roller table rollers 38 at the rear end of the machine are provided with bevelled gears 39 which also cooperate with bevelled gears 40 carried on the main drive shaft 8. The periphery of the roller table rollers 38 is so proportioned to the speed of the molds that the speed of the periphery of these rollers is exactly the same as the speed of travel of the mold trough.

In connection with continuous slabs of certain predetermined cross section to be delivered from the apparatus, it may be desirable to roll the edges, and therefore edging rolls 41 are provided adjacent the end of the upper run of the continuous mold trough. These edging rolls may be dispensed with under certain conditions. It is to be understood that where the rolls 41 are used, there are at least two edging rolls 41 one on each side of the slab (only one edging roll being shown in Fig. 1). Under certain conditions, surfacing rolls may also be desirable and a pair or more of surfacing rolls 42 and 44 are provided where these rolls are desirable. Both the edging rolls 41 and the surfacing rolls 42 and 44 are power driven at the proper speed relative to the travel of the continuous slab.

While the machine is adapted for continuous operation, and the continuous slab may be run directly into a rolling mill, it is sometimes desirable that individual lengths shall be severed from the slab and therefore a pair of flying shears 45 is provided. The shears have a movement with the slab during cutting. However, the preferred operation is that the continuous slab shall run directly into a continuous rolling mill 46 comprising a plurality of roll stands.

It may be desirable to spray the molds with water and therefore, a water spray 47 may be provided at the rear end of the machine to spray the molds while hot. It is also desirable in some cases to spray the molds with treatment compounds such as tar, graphite mixtures, etc., and where this is desired, a spraying apparatus 48 is provided adjacent the forward end of the mold chain to apply such treatment mixture.

Referring now more especially to Figs. 3 and 4 which illustrate in more detail the continuous mold trough, the individual mold members 4 preferably are provided with a pair of link arms 49 on one end of each mold member, and another pair of link arms 50 at the other end of each of the individual mold members. The link arms 50 have their forward ends offset in order to fit within the

70

75

80

85

90

95

100

105

110

115

120

125

130

link arms 49 of an adjacent mold member. These link arms preferably are provided with slots through which key bolts 51 are adapted to be passed in order to form the individual 5 mold members 4 into a continuous chain and to permit expansion and contraction of the mold members without stress on the coupling means.

Referring now more especially to Figs. 5, 10 6, and 7 which represent the cap members, these members have their sides cut away as at 52 and 54 to provide projecting edges 55 and also a downwardly projecting member 56 which is adapted to fit into the trough 15 mold members 4. The cap members are provided with a pair of link arms 57 on one end and another pair of link arms 58 on the other end. The link arms 58 are offset to fit within the link arms 57 and these arms are also 20 slotted at 59 for the same purpose as in the mold chain.

In carrying out the method of the present invention, the steel is poured from a ladle 59 upon a continuous mold trough 3 to form a 25 pool. In the initial start of the device, a temporary dam 60 is set in the mold trough to provide a small initial pool between the main dam 21 and the temporary dam 60. This temporary dam 60 is illustrated in Fig. 30 1 as being raised above the mold trough and is ready to be dropped into position when necessary. As soon as a pool has been formed substantially equal to the height of the temporary dam 60, the machine is started and 35 the stream of steel from the ladle 59 is continued at a sufficient rate to maintain the height of the metal about level while the trough is moving in the direction of the arrow A (Fig. 1). This causes the pool to 40 elongate and causes the temporary dam to pass under the moving continuous cap chain. As the cold chill caps touch the cap of the molten pool, these caps form a skin on top of this molten steel; which skin continues to 45 thicken so as to form a substantially tubular condition of chilled steel enclosing a molten core. When the machine is in full operation, this molten core extends partly under the continuous caps, gradually becoming smaller 50 and thinner until finally the molten core has completely been replaced by solid metal. The molten metal is indicated in Fig. 1 as at M and the solid metal is indicated at S. The speed of the machine is maintained sufficiently high 55 to enable the caps and the molds to completely chill the steel so that it leaves the end of the cap continuous chain as a solid continuous metal slab. The dam 21 prevents the steel from running out of the forward end of the 60 machine and since this dam sits close to the molds, there is no tendency of the metal to flow back between the dam and the molds in view of the fact that the molds are moving forward and the metal is being chilled between the dam and the mold members, thus

this dam 21 forms an effective head to maintain the pool of liquid molten steel, which pool is continuously replenished and continuously carried away by the molds and the caps as fast as molten steel is supplied to the machine. It will be observed that the caps are gradually pressed down into the molds during the time when the steel in the molds is gradually freezing so that the metal preferably may be compressed during freezing and the continuous slab issues as a perfectly solid piece of steel. For some conditions, it may be desirable to force the caps full down when the caps first touch the liquid steel. This may be done by adjusting the axes of the rollers 31 parallel to the run of the mold trough 4. It will also be observed that the open pool between the dam 21 and the drive wheel 25 is of sufficient length to permit the full escape of gas from this shallow pool of molten steel so that by the time the cold chill caps come on to the steel, the gasification thereof has practically ceased. Since the pool is of molten steel relatively thin and is continuously moving through the machine, it will be observed that segregation of the steel constituents is substantially prevented so that the slab of steel coming from the apparatus is uniform in character, solid in physical aspects and of exactly the right shape for the rolling mill. It will also be observed that by changing the face contour of the molds and the caps that various cross sectional shapes such as an hourglass or a substantially curved shape, oval in cross section may be produced. This permits the shaping of the continuous slab to suit the requirements of the rolling mill.

Figs. 8 to 11 of the drawings illustrate a few of the many cross sectional shapes which may be formed by shaping the bottom of the mold and the under face of the cap so that a predetermined cross section will be given to the continuous slab. The shape 61 shown in section in Fig. 8 is best adapted to the making of plates and flat bars. The shape 62 in Fig. 9 is well adapted for rails and such like forms. Figs. 10 and 11 illustrate cross sections through the caps and the molds wherein the metal in the molds and in the caps are distributed in such manner as to cause uniform chilling of the cross section of the slab of steel. The molds 4a and 4b and also the caps 24a and 24b illustrated in these Figs. 10 and 11 have the heat absorbing capacity of the metal chill arranged opposite to the largest mass of molten steel in the continuous slab cross section. The shape 64 illustrated in Fig. 10 is adapted for certain types of I-beams and the shape 65 illustrated in Fig. 11 is adapted for certain oval structures or round bars, rods, etc.

Referring now more especially to Figs. 13, 14 and 15, there are certain types of molten steel where it may not be necessary or desir-

able to cap the top surface of the continuous slab, especially where it is not necessary or desirable to shape the top of this slab for subsequent fabrication. In this form the method may be carried out in an apparatus comprising a substantially continuous open trough mold. Such a structure is diagrammatically illustrated in Figs. 13 and 14 wherein a continuous mold bottom 66 is mounted upon a drive wheel 67 at one end and an idler wheel 68 at the other end. Supporting rolls, driving devices, and other mechanisms are omitted in order to simplify the disclosure. The upper run of the bottom 10 of the mold makes an incline as at 69 and this incline extends above the height of the molten metal pool which will be formed in the apparatus. In this form of apparatus, the sides of the mold preferably comprise side 15 chain members 70 and 71 which are identical in form and are arranged on each side of the upper run of the mold bottom chain 66. These side members preferably are provided with anti-friction rollers or wheels 72 mounted on the shaft 74 (Fig. 15) between the connecting link arms 75 and 76 which are suitably riveted or otherwise secured to the side members 70 and 71. These rollers 72 are adapted to run against a rail 77 which is provided with screw supports 78 constructed to force the rail against the inner run of the chain sides and thereby force these side members 70 and 71 against the edges of the upper run of the mold bottoms 66 to make a tight 20 contact and form a long travelling trough. In this form of apparatus as illustrated in Figs. 13 and 14, the caps have been omitted and the trough is of sufficient length to permit the solidification of the steel without 25 necessity for capping. In other words, the bottom and sides of the mold trough are of sufficient weight and size to cause the metal to freeze from the bottom upwardly, so that the slab as it leaves the machine is completely 30 frozen. The side members and the bottom members are driven at exactly the same linear speed and are driven from the forward end of the machine, like a locomotive pushing a train of cars, thereby pressing the joints between the individual sections tightly together 35 to prevent steel fins forming in the joints.

In connection with the operation of the device, it will be observed that the main drive shaft 1 is located at the forward end of the 40 machine and that the driving of the mold members is progressive from the forward end, so that the mold members are tightly butted together in the upper run of the mold chain, in the same manner as a locomotive pushing a train of cars. This causes the joints between the mold members to be tightly pressed together and since the molds are cold, there is no tendency of molten steel 45 escaping from these joints. The same driving condition occurs in connection with the

continuous caps which close the tops of the molds to form a substantially tubular mold zone so that there is no tendency of the liquid steel rising in the joints between the caps.

In the preferred operation of the present device, a ladle is used which is of such capacity as to take the entire output of one furnace cast and the temporary dam is placed in the molds and the casting operation is continued until the entire contents of the ladle have run through the machine and when the ladle has finished pouring, another temporary dam 60 is dropped into the mold trough adjacent permanent dam 21. This temporary dam 60 now comprises a travelling head which holds the pool of molten steel from thinning out into a thin layer and permits the machine to run clean for the end of the ladle pour, thereby greatly reducing waste and utilizing substantially all of the metal from the ladle. After one furnace cast has been completed, the operation is repeated with the next furnace cast starting with the temporary dam 60 as previously explained. If it should be desired to have continuous operations a new ladle may be poured into the machine to form a new pool back of the temporary dam 60 as it moves forward. This dam 60 then acts to separate the furnace charges, or if the several charges of the different furnaces are sufficiently uniform in character the dam 60 may be omitted between ladles providing the new ladle is brought up before the pool has lessened perceptibly in height.

In the present method, it will be observed that a pool of molten steel of substantially uniform depth is maintained by adding molten steel to the pool while draining it at one side by gradually and continuously moving the pool supporting members in one direction and freezing the steel in the pool supporting members as they move away from the pool. This frozen steel is carried away at substantially the same rate as molten steel is supplied to the pool so that the operation is in effect a continuous moving body of steel of a predetermined volume, which body is molten at one end and solidified at the other, whereby a continuous stream of steel issues through the machine with the stream being molten at one end and solidified and shaped at the other end of the machine.

The term "continuous casting" as used herein and in the claims means casting continuously for a relatively long period of time either from a single ladle or a plurality of ladles or in any other manner; and this term also implies casting from single ladles with a complete stoppage of casting operations between each ladle full of metal.

The term "continuous shapes" is used to mean shapes which heretofore in the art have been made by working ingots down to the point where the final fabricating opera-

tions begin such as rolling or forging or wire drawing or other fabricating operations. In other words, the present method and apparatus is adapted for the production of metal masses directly from molten steel or other metals and so shaped as to be immediately ready for the final fabricating operations. It is also to be understood, however, that where desired the present method and apparatus may produce such shapes as may undergo an intermediate step or steps of operations prior to the final fabricating step.

The term "steel" used herein is intended to mean iron or any iron alloy or compound heretofore commonly cast into ingots and worked from ingots into final form through a plurality of intermediate step operations.

It is also to be understood that where desired heating furnaces such as electrical or gas furnaces or any other type of heating device may be used, as is common in the art, to heat the metal after it has been initially solidified and during the subsequent treatment.

Having described our invention, what we claim is:

1. The method of preparing a mass of metal for rolling operations which comprises forming a pool of molten metal, progressively lengthening the mass of metal by adding molten metal to one end thereof, cooling the metal progressively from the metal initially placed in the pool to the metal progressively added to form a frozen elongated mass, and applying lateral pressure to the metal during the freezing thereof.

2. The method of preparing a mass of metal for direct fabrication which comprises forming an elongated mass of metal frozen at one end and molten at the other end by progressively moving the metal and by continuously pouring molten metal into the molten end of the mass and simultaneously withdrawing heat from and applying pressure to the metal between the ends of the mass before the freezing action is completed.

3. The method of preparing metal for rolling operations which comprises forming an elongated slab of metal solid at one end and molten at the other by continuously pouring molten metal at the molten end, continuously moving the poured metal away, and allowing it to solidify; and applying pressure laterally of the slab while the metal is still soft.

4. The method of preparing metal for fabricating operations which comprises forming an elongated slab of metal solid at one end and molten at the other by continuously pouring molten metal at the molten end, continuously moving the poured metal away, and allowing it to solidify; and pressing the slab into a desired cross sectional shape while the metal is still soft.

5. The method of preparing metal for roll-

ing operations which comprises progressively pouring molten steel into an elongated trough-shaped mold from one end of the trough to the other, allowing the metal to progressively cool in the trough to form a slab of metal solid at one end and molten at the other, with an envelope of frozen metal between said ends enclosing a wedge-shaped mass of molten metal, applying lateral pressure to the slab adjacent the small end of the wedge-shaped mass, and progressively removing the solidified metal from the mold.

6. The method of preparing metal for rolling operations which comprises progressively pouring molten metal into an elongated trough-shaped mold, permitting the metal to progressively solidify to form an elongated slab of metal solid at one end and molten at the other, and progressively applying lateral pressure to a portion of the slab which is still soft in the mold.

7. The method of preparing metal for rolling operations which comprises progressively pouring molten metal into an elongated trough-shaped mold, permitting the metal to progressively solidify to form an elongated slab of metal solid at one end and molten at the other, progressively applying lateral pressure to a portion of the slab which is still soft in the mold, and progressively removing the solidified metal from the mold after lateral pressure has been applied thereto.

8. The method of continuously casting shapes for immediate rolling operations, which comprises discharging a stream of molten steel into a substantially horizontal mold, producing relative movement between the stream and the mold, said movement being longitudinal of the mold, progressively chilling the stream to form an envelope of frozen steel enclosing a wedge-shaped mass of molten steel adjacent the head of the stream, and applying pressure to said wedge-shaped mass and supporting the envelope to prevent rupture.

9. The method of casting continuous slabs of steel comprising, maintaining a moving stream of molten steel, supporting and moving the stream upon chill molds, applying lateral pressure to the stream to maintain the stream in contact with said chill molds during the movement of the stream until the foot end of the stream is completely frozen, and adding molten steel to the head of the stream to maintain the stream substantially constant.

10. The method of continuously casting molten steel shapes for subsequent fabrication comprising, maintaining a stream of steel, chilling the stream of steel progressively from the foot of the stream to the head thereof so that the foot of the stream is frozen solid while the head of the stream is substantially liquid, progressively applying

- lateral pressure before the freezing action is completed, and supplying molten steel at the head of the stream to maintain the stream substantially uniform.
- 5 11. The method of continuous casting of metal shapes ready for subsequent fabrication, which method comprises withdrawing the heat from a stream of molten steel at such rate that the foot of said stream comprises 10 completely solidified metal while the head of said stream is substantially molten metal with a frozen envelope enclosing a mass of partially frozen steel, applying pressure to said partially frozen steel, and completely 15 supporting said envelope to prevent rupture, causing said stream to move from the molten head toward the solid foot, and supplying molten metal to the head of said stream to maintain the same at substantially 20 uniform depth during casting operations.
12. The method of continuously casting shapes from molten metal which shapes are ready for subsequent fabrication comprising a moving stream of molten metal, withdrawing heat from the entire circumference 25 of said stream as it moves so that the foot of said stream is solid frozen metal applying pressure to a portion of said stream during the moving thereof to compact a portion of 30 the metal of said stream into a solid mass of predetermined cross section.
13. The method of continuously casting steel shapes of predetermined cross section from molten steel comprising moving a 35 stream of molten steel by moving chill molds which support said stream at the rate at which the stream moves, chilling the surface of a portion of said stream whereby the head of said stream is an open pool of molten 40 steel and the foot of said stream is solid steel of a predetermined cross section and an intermediate portion of the stream is in the form of a frozen steel envelope surrounding a molten steel core which gradually increases in size from the solid portion of the 45 steel toward the open molten pool, and supporting said envelope against rupture while applying lateral pressure to the envelope.
14. The method of casting continuous steel 50 shapes of predetermined cross section comprising maintaining a moving stream of steel having at one end an open pool of molten steel and at the other end a solid frozen steel mass of predetermined cross section and compressing the intermediate soft partially frozen steel prior to fabricating operations.
15. The method of casting continuous 55 shapes from molten steel comprising moving a stream of steel by moving a continuous chill bed for said stream at the rate of movement of said stream, maintaining an open pool at the head of the stream, chilling all sides of the stream between said open pool and the foot of the stream to form a frozen envelope 60 enclosing molten steel, and supporting said

envelope while applying lateral pressure to the envelope, whereby the foot of the stream comprises a continuous solid mass of predetermined cross section.

16. An apparatus for continuously casting steel shapes of predetermined cross section comprising an open trough chill mold member, means to prevent molten steel from running out of the head of said trough, means to move said trough, and covering means being adapted to enter into said trough, said covering means being spaced from the head of said trough to maintain an open space in which an open pool of molten steel may form, said covering means being adapted to travel at the same rate as said mold member and to chill the upper portion of steel in said mold member.

17. In an apparatus for casting continuous shapes of predetermined cross section from molten steel comprising traveling means adapted to support and chill the under portion of the sides and a stream of steel, and capping members adapted to enter into said means to shape, to compress, and to chill the upper portion of the steel in said means.

18. An apparatus for continuous casting of steel shapes of predetermined cross section for immediate rolling comprising a continuous chain of open ended horizontal chill molds, means to drive said chain, capping means for a portion of said chain and adapted to fit into said horizontal molds and to come in contact with steel within said horizontal molds, and pressure means to force a portion of said capping means into said molds.

19. An apparatus for casting predetermined shapes from molten steel, said apparatus comprising a continuous traveling chill mold member of sufficient heat absorbing capacity and of sufficient length to substantially chill molten steel poured into said member, means to drive said member at such rate as to permit the freezing of said steel in said member before the steel leaves said member, means to apply lateral pressure to the steel while still soft and before the steel leaves said member, and a continuous rolling mill to fabricate said frozen steel in final form.

20. In an apparatus of the class described, 115 a series of trough-shaped mold sections fastened together in an endless chain, means to move said mold sections to form a substantially horizontal trough-shape mold traveling lengthwise of itself, cap members adapted to move into said mold sections, means to discharge a stream of molten steel into said trough-shape mold while the same is in motion, and means to apply pressure to said cap members to compress the steel within said mold.

21. In an apparatus of the class described, means forming an elongated trough-shape mold, driving means to move said mold lengthwise of itself to carry forward molten

metal being fed into said mold to form an elongated metal slab in said mold, and means to apply lateral pressure to a portion of the slab while in said mold.

- 5 22. In an apparatus of the class described, a series of trough-shape mold sections connected into an endless chain, means to drive said chain of mold sections to form a substantially horizontal trough-shaped mold 10 moving continuously lengthwise of itself, roller means to support said trough-shaped mold, means to discharge a stream of molten metal into said trough-shaped mold to form a slab of metal therein, and movable means 15 to apply lateral pressure to said slab of metal in said mold.

23. In an apparatus of the class described, a series of trough-shaped mold sections connected together to form an elongated trough-shaped mold, means to move said mold lengthwise of itself, means to discharge a stream of molten metal into said mold while the mold is in motion to form a slab of metal in said mold, and means moving with the mold to apply 20 pressure to the upper surface of said slab of metal and chill the same.

24. In an apparatus of the class described; a series of horizontal open ended chill mold members; means to secure a plurality of said 30 chill mold members together end to end, said means permitting expansion and contraction of the chill mold members; and means to move said series of chill mold members by causing one mold member to push the one in front of 35 it to maintain molten steel tight joints between said chill mold members.

25. In a device of the class described, the combination of a long trough horizontal chill mold, means to discharge a stream of steel 40 into said mold, means to cause a relative longitudinal movement between said stream and said mold during pouring operations, means to circumferentially chill said stream, and means to support and apply pressure to 45 a portion of said stream during chilling thereof.

26. A machine of the class described adapted to cast continuous steel billets, comprising a plurality of mold sections in the 50 form of a travelling chain, means to drive said chain, means to guide certain of said mold sections in substantially a straight line where said sections are adapted to support said steel billet, and means to remove said 55 mold sections from said steel billet without any portion of said removed sections exerting pressure against said billet when the sections are being removed from the billet.

27. In a device of the class described, the 60 combination of a plurality of mold members comprising sections of a continuous travelling chain, means to drive said chain, means to guide said mold sections whereby a portion of said chain comprises a substantially 65 straight run, and means to guide said mold

sections away from said straight run in such manner that the mold sections are taken away with all portions thereof below the line of straight run.

28. A continuous billet casting machine 70 comprising a plurality of open ended trough chill molds arranged end to end to comprise an elongated mold member, means to pour molten steel into one end of said mold member, the sides of said molds being of such 75 height as to be at all times above the highest part of the molten steel in said mold, chill cover members movable into said mold member and resting on molten steel therein and being adapted to chill the molten steel in 80 said mold member, and means to push said molds and said cover members endwise.

29. The method of continuously fabricating steel shapes comprising casting a continuous billet of steel, applying pressure to the 85 billet during casting, moving the steel billet to a rolling mill, and rolling one end of the continuous billet while the other end of the billet is being cast.

30. The method of fabricating steel shapes 90 comprising casting a continuous steel billet with one end thereof being molten metal and the other end being frozen metal, applying lateral pressure to the billet adjacent the molten end and rolling the frozen metal to 95 shape the same.

31. The method of continuously fabricating steel shapes comprising forming a moving stream of steel, adding molten metal to one end of said stream to maintain the cross 100 section of said stream substantially constant, progressively chilling a portion of said stream, applying lateral pressure to a portion of the stream during the chilling thereof and rolling the metal from the chilled portion. 105

JOHN E. PERRY.  
GEORGE RAMSEY.

110

115

120

125